

# UNITED STATES PATENT OFFICE.

ROLLIN H. WIGGIN, OF EAST ORANGE, NEW JERSEY, ASSIGNOR TO H. B. WIGGIN'S SONS COMPANY, OF BLOOMFIELD, NEW JERSEY, A CORPORATION OF NEW JERSEY.

## PROCESS OF PRODUCING WALL-COVERING AND PRODUCT THEREOF.

1,313,658.

Specification of Letters Patent.

Patented Aug. 19, 1919.

No Drawing.

Application filed September 9, 1915. Serial No. 49,682.

*To all whom it may concern:*

Be it known that I, ROLLIN H. WIGGIN, of East Orange, in the county of Essex, and in the State of New Jersey, have invented a 5 certain new and useful Improvement in Process of Producing Wall-Covering and Product Thereof, and do hereby declare that the following is a full, clear and exact description thereof.

10 The object of my invention has been to provide a fabric wall covering which shall be water-resisting, and a process of making the same, which shall have, among others, the following advantages: that of enabling 15 the fabric to be made either with its natural texture or with a filled surface; that of enabling the face of the goods to be thoroughly water-resisting while leaving the back of the goods sufficiently water-soluble; that of employing only aqueous solutions of the water- 20 proofing substances, and specifically that of employing an albuminoid substance rendered insoluble by the action of formaldehyde, and an insoluble softening agent, such as an insoluble soap or linseed oil, and to 25 such ends my invention consists in the water-resisting fabric and process of making the same hereinafter specified.

My invention is capable of embodiment 30 in many different forms, and while I shall describe that embodiment which is the best one known to me, it is to be taken as illustrative only of many possible embodiments.

In the illustrated embodiment, I use a 35 strip of cotton cloth but may use any suitable fabric. I wish to make the fabric water-resisting so that, for instance, it can be cleaned, and do so by treatment with an albuminoid substance, rendered insoluble by 40 the action of formaldehyde, and an insoluble softening agent such as an insoluble soap or linseed oil.

In the particular instance chosen for illustration, the process of making the fabric 45 is as follows:

The fabric is run through various machines common in the art of treating fabrics, and for convenience I shall refer to the various passages of the goods through the 50 machines as "Run No. 1," etc. The fabric is first given a dip run on a padding ma-

chine. An example of a mixture suitable for use on the first run is as follows:

|                                         |    |
|-----------------------------------------|----|
| 56 lbs. clay mixture made up of 28 lbs. | 55 |
| clay and 28 lbs. water.                 |    |
| 64 " water                              |    |
| 9 " wheat flour                         |    |
| 2 " glue                                |    |
| 8 " water                               | 60 |
| Preservative                            |    |
| Coloring matter.                        |    |

The mixture is made as follows: 28 lbs. of clay is mixed with 28 lbs. of water; 9 lbs. of flour is mixed with 64 lbs. of water; 2 lbs. of glue is mixed with 8 lbs. of water and brought to a boil. The whole is then mixed and cooked until homogeneous. The object of this run is to decrease the absorption of 70 the fabric, making the foundation for the other runs.

The second run is through a coating machine by which a filling run is applied to the face of the goods, the object being 75 to fill up the interstices between the threads. A suitable mixture for this run is as follows:

|                                      |    |
|--------------------------------------|----|
| 68 lbs. clay mixture made by soaking |    |
| equal amounts of clay and water      | 80 |
| 16 " water                           |    |
| 10 " corn starch                     |    |
| 10 " wheat flour                     |    |
| 16 " of a solution made by boiling 1 |    |
| part, by weight, of linseed with 85  |    |
| 16 parts, by weight, of water        |    |
| and straining off the undissolved    |    |
| portion.                             |    |
| 20 " of casein solution made by dis- |    |
| solving one part, by weight, of 90   |    |
| casein in four parts, by weight,     |    |
| of dilute ammonia.                   |    |
| 10 " of mixture made as follows, and |    |
| which may be called the "oil         |    |
| mixture."                            | 95 |
| 4 " casein (dry)                     |    |
| 10 " lithographic varnish            |    |
| 10 " hot water                       |    |
| 5 " ammonia.                         |    |

In making the mixture, mix the casein 100 with  $2\frac{1}{2}$  lbs. ammonia and 5 lbs. water, and heat. Mix the lithographic varnish with

2½ lbs. ammonia and 5 lbs. of water and heat; then mix the two and stir until homogeneous.

Coloring matter

5 Heat and stir the whole until homogeneous.

The third run is a repetition of the second run.

10 The fourth and fifth runs are made on a printing machine and are for the purpose of applying a finishing coat containing an albuminoid such as casein, glue, albumen or possibly gluten, and a soluble softener. When the albuminoid is rendered insoluble, 15 as later described, it becomes too brittle and hard, and the function of the softening agent, such as an insoluble soap or linseed oil, is to introduce an insoluble softening agent to overcome the brittleness of the insoluble albuminoid substance. I desire to 20 get the substances into the cloth in a condition soluble in water so as to avoid the use of inflammable solvents, and then to render them insoluble after the fabric has 25 either been coated or impregnated with these substances.

A suitable composition for the fourth and fifth runs is as follows:

30 17 lbs. 8 oz. of oil mixture, as above,  
1 " 12 " of alcohol,  
1 " 12 " of water (hot).

Suitable amount of coloring matter either dye or pigment.

35 The sixth run, when used, is the printing of a design upon the fabric, and is applied by a printing machine. A suitable mixture for the printing run is as follows:

40 10 lbs. of oil mixture, as above,  
2 " alcohol  
— dyestuff or other coloring matter.

The seventh run is, or may be, the application of a solution which renders insoluble 45 the albuminoid and softening agents put on by the printer. A suitable mixture for this purpose is as follows:

50 20 lbs. water,  
1 " 40% formaldehyde,  
8 oz. sulfate of alumina.

The eighth run is to put a backing upon the back of the fabric. This is accomplished 55 on a coating machine. Any well-known composition may be used as my invention does not relate specifically to it. The object of the backing is to cause the fabric to adhere to a wall when pasted with flour 60 paste or other suitable adhesive.

Between each two runs the goods are dried, as over cylinders heated by steam.

It will be noted that in the compositions 65 used for the first six runs an albuminoid substance is present. For instance, in the

first run there is glue or casein present as an albuminoid substance.

In the second, third, fourth, fifth, and sixth runs there is a soluble soap formed by the lithographic varnish (which is boiled 70 linseed oil) mixed with ammonia.

In the seventh run the formaldehyde renders the albuminoid substance insoluble and the sulfate of alumina renders the soluble soap insoluble. Any insoluble soap, such 75 as lead soap or magnesia soap can be used as well as that found in the above formulae, and any suitable soluble soap can be used and rendered insoluble by the use of any suitable water-soluble precipitant. 80

In the composition for the second, third, fourth, fifth and sixth runs, linseed oil can be used which has not been saponified, but in that event the alum or sulfate of alumina would be omitted from the seventh run. 85

My above described fabric and the process of making the same, have, among others, the following advantages: The fabric is water-resisting so that it can be cleaned. In the process of making it, the use of inflammable 90 solvents is avoided. The water-resisting quality is sufficiently perfect for all practical purposes on the exposed face of the goods, and yet the portions of the fabric toward the back are not so insoluble that 95 a backing which would take hold of flour paste or other water soluble adhesive on the wall cannot penetrate the goods and take hold of them. The fabric is coated or impregnated with the substances which render 100 it waterproof by the use of water solutions carrying said substances, and the said substances are then rendered waterproof *in situ*. By the term "insoluble" as used in 105 the specification is meant substantially insoluble in water. By the term "water-soluble" and similar terms is meant capable of being carried in water as a vehicle, whether literally soluble or only in suspension. 110

Applicant throughout his specification and 110 claims intends the terms "proteid" and "albuminoid" as having the same meaning.

I claim:

1. A fabric having a water-resisting face, and a water-absorbent back, the body of 115 the fabric in between said face and back increasing in water-solubility from the face to the back.

2. A fabric wall covering having a water-resisting face, and a water-absorbent back, 120 the body of the fabric in between said face and back, increasing in water-solubility from the face to the back.

3. A process of producing a fabric having 125 a water-resisting surface, comprising impregnating said fabric with an aqueous solution of an albuminoid substance and with a soluble soap, and rendering said albuminoid substance insoluble with a solution of formaldehyde and said soap insol- 130

ble with an aqueous solution of a water-soluble metallic salt.

4. A process of producing a fabric having a water-resisting surface, comprising 5 impregnating said fabric with an aqueous solution of an albuminoid substance and with a soluble soap, and rendering said albuminoid substance insoluble with a solution of formaldehyde and said soap insoluble with an aqueous solution of a water-soluble metallic salt such as sulfate of alumina.

5. The process which comprises treating a fabric with a solution containing an albuminoid and a soluble soap, subjecting the 15 treated fabric to the action of a formaldehyde solution and rendering the soap insoluble.

6. The process which comprises treating a fabric with a solution containing an al- 20 buminoi and a soluble soap, and subjecting the treated fabric to the action of a solution containing formaldehyde and a water-soluble metallic salt.

7. The process which comprises treating 25 a fabric with an albuminous solution containing casein and also containing a soluble soap, then subjecting the treated fabric to the action of a formaldehyde solution and rendering the soap insoluble.

In testimony that I claim the foregoing I have hereunto set my hand.

ROLLIN H. WIGGIN.

Witnesses:

JOHN R. WINANS,  
ANGELA C. BURKE.